

Feb. 24, 1959

J. R. EHRLICH

2,875,101

RUBBER COATED WOOD

Filed July 29, 1954



FIG. 1



FIG. 2



FIG. 3

INVENTOR.

Joseph R. Ehrlich.

BY

Maxwell E. Sparrow.

ATTORNEY.

1

2,875,101

**RUBBER COATED WOOD**

Joseph R. Ehrlich, New York, N. Y.

Application July 29, 1954, Serial No. 446,669

3 Claims. (Cl. 117—148)

This invention relates to article of manufacture comprising at least two members which are cohesively but not coalescingly attachable to each other, and the method of treating the body or base of each of such members to impart such quality to the same.

I have discovered that wood pieces or members treated according to this invention can be made to adhere to each other temporarily by simply touching their surfaces together; and that such members can be taken apart again and put together again, repeating that procedure over and over again without the members losing their property of adhesion and without the members adhering to any other surface than their own or members having similar surfaces, and without the surfaces of such members exhibiting any stickiness or tack to the touch. Such treated wood members have no surface tack, that is, they are not tacky, adhere strongly to each other and the members may be separated without injury to their surfaces. An important feature is that the skins of the respective members when the latter are brought together adhere to each other without any coalescent action. In the manner of the present invention, smoothness, resilience, flexibility and tautness of the skin enable the contacting members to touch each other completely and without any space between the contacting surfaces; and the adhesion of the skins to their respective wood bases is stronger than the cohesion developed between the said skins when the members are brought together.

It is an object of the present invention to provide an assembly comprising at least two members treated in such a manner that they may be made to engage each other by touching their surfaces together through cohesive attraction and not coalescence and which are then readily disengageable without destroying or injuring the engaging surfaces.

It is another object of the present invention to provide an article of manufacture comprising a plurality of wood elements the surfaces of which are capable of absorbing moisture, and a casing completely covering each of the elements, the casing consisting of a flexible, non-tacky, non-coalescing, resilient and elastic skin tightly shrunk on the element, the casings being adapted when the elements are brought together under slight pressure to cohere without tack or coalescence and being readily and repeatedly separable from each other without separating from their respective elements.

It is still another object of the present invention to make the skins in the form of a transparent film.

Yet another object of the present invention resides in the method of making or producing such articles.

These and other objects and advantages of the invention will appear as the description proceeds, it being understood, however, that it is not intended that the invention be limited to the exact details described herein which

2

illustrates the production of some satisfactory products of many which may be obtained as a result of the knowledge gained through or gleaned from an understanding of the invention; and it is further intended that there be included, as part of the invention all such obvious changes and modifications thereof as would occur to a person skilled in the art to which this invention pertains and as would fall within the scope of the claims.

In the drawings:

- 10 Fig. 1 is a perspective view, partly in section of a wooden piece according to the invention;  
Fig. 2 is a sectional view taken on line 2—2 of Fig. 1; and  
Fig. 3 is a much enlarged end view of two wooden pieces shown in Fig. 1, in the process of being separated by hands.

In order to impart to the articles the aforementioned properties, it is important for best results to select wood members having moisture absorbing surfaces, that is, the surfaces of the wood members should be porous, not covered with varnish, lacquer or other sealing material. These wood pieces or members are each encased completely with a non-tacky, tight-fitting, elastic, flexible, shrinkable and resilient skin which is preferably thin, transparent, non-visible and hardly noticeable. This skin is solidly and completely anchored to the wood member or base as long as the casing is complete, uninjured and has no loose ends.

Pressure sensitive adhesives commonly in use at present are permanently tacky without being moistened and adhere to any non-tacky, dry surface under light pressure, and can easily be removed therefrom without any traces left on the applied surface. However, if the tacky surfaces of the articles to which the pressure sensitive adhesive is applied are brought into contact with each other, the two surfaces will not merely cohere but will coalesce and cannot be readily pulled apart without injury to the surfaces. In other words, these contacting surfaces due to coalescence, will have to be virtually torn apart in order to separate them from each other.

There are well known self-sealing adhesives which are non-tacky, do not adhere to dry, non-tacky surfaces, but coalesce, however, if pressed together. Such dry adhesives are used, for example, in the shoe and envelope-making industries. However, when such surfaces are pressed together they produce strong and permanent bonds and the members having such adhesive surfaces cannot be pulled apart without at least impairment to or peeling off of the skins forming the adhesive coatings or surfaces and, in fact, in many instances, injuring the fibers of the members to which the adhesive is applied.

In the practice of the present invention, the two types of adhesives just referred to are definitely to be avoided. The type of adhesive employed to form a skin encasing the wooden members must be non-tacky, must form a skin or surface which will not adhere to any skin or surface except to a skin or surface of the same kind, must form a skin which is elastic, flexible, non-tacky, shrinkable, resilient and tight-fitting and so strongly anchorable to its base or member, that contact and separation of the bonded surfaces can be repeated many times without injury to the surfaces, and the skins or surfaces remain dry and clean after each separation. It has been found that an adhesive comprising a non-vulcanized rubber interspersed with particles of film-forming material that breaks the coalescence of the surfaces or skins when formed, that is, that prevents coalescence of the skins, satisfies the foregoing requirements.

As an example of carrying out the invention, in neatly cut pieces or members of wood with a smooth, but absorbent surface, non-rusting clean pins are driven into one far end of the pieces or members about one-eighth inch deep. These pinned wooden members are dipped into the dipping solution so that they are completely immersed and deep enough that about one-eighth inch of the free end of the pin is also immersed. The solution forms a substantially white coating which turns transparent when dry. To remove the pin, the wooden member is pulled down straight. The skin covering the lower part of the pin slides off the pin easily, provided that the latter was clean before dipping. This little protruding part of the skin contracts immediately and closes over the tiny hole caused by the insertion of the pin. Thus, the wooden piece or member is totally and completely encased by the skin, and the latter is anchored to the wood.

Another method of producing an endless casing, that is, a casing without free or loose ends where peeling could possibly start, is by performing the dipping operation in two steps, namely, dipping one portion first in the solution, then permitting this portion to dry completely to form a skin; then turning the member around and dipping the other, undipped portion in the solution in such a manner that the second dip slightly overlaps the first dipped portion and then permitting the second dipped portion to dry; thus now forming a completely sealed and endless skin over all of the surfaces of the member without any loose ends or edges.

The dipping liquid or solution may comprise, for example, a blend of two-thirds of a water solution containing 5% by weight of water-soluble methylcellulose and one-third of a natural rubber latex of 38% to 40% by weight of solid contents. The methylcellulose should be of low viscosity, e. g. five to fifteen cps. The blend should have a pH not less than 8.5, and may or may not contain de-foaming agents, wetting agents, anti-oxidants or other additives. The latex dispersion in the methylcellulose solution is not stable and has a tendency to separate. Therefore, high speed agitation before dipping is necessary in order to have the methylcellulose well interspersed within the dry rubber skin. In the preceding example, the ratio of solid methylcellulose to solid rubber in the dry skin can be calculated to be between 1 to 3.8 to 1 to 4. Depending upon the type of latex employed, the manner in which it was processed, etc., it might be necessary to change the ratio of the solid contents of the components in the dry skin. Using a 60% centrifuged latex, water will have to be added to the blend and the ratio of methylcellulose to rubber might be 1 to 6.

It is preferred to use methylcellulose because it strengthens the rubber skin more than other film-forming additives which likewise would prevent tack and coalescence of the rubber skin. However, there can also be used sodium carboxy methylcellulose, hydroxy ethylcellulose, carboxy methyl hydroxy ethylcellulose, water soluble metal poly acrylates and other non-tacky water soluble, film-forming materials in whose water solutions or dispersions latex is dispersible without coagulation.

The skin or casing as produced in the aforesaid examples, has no cold flow, is non-tacky to the touch and does not adhere to any other surface but one of its own type. When it adheres to its own surface, it does not coalesce as a plain non-vulcanized rubber skin might do; such coalescence does not take place at room temperature, and not even over any extended period of time or under moderate pressure. Any pressure-sensitive adhesive of any denomination, or self-sealing adhesive or heat sealing adhesive would coalesce under the aforementioned conditions. Neither could any such adhesive skins or surfaces be separated from each other without causing injury to the skin or film, or without being pulled off its base, wholly or in part. The encased wooden pieces or members must have the property to be capable of adhering to each other and be separated over and over again without

any injury to the skin encasing the member and as often as desired, regardless of season or atmospheric conditions and over a long period of time.

Articles made according to the invention may be employed for several purposes and uses, for example, construction toys, model furniture, houses, machines and other objects. These articles or members may also be used to form letters, figures, etc., for educational as well as for window display purposes and also for constructing anatomical models. The parts or members may be taken apart, rearranged, or reassembled as frequently as it is desired. The members may further be used to temporarily adhere one to another when made in the form of game pieces or to a board upon which the game is played.

Figs. 1 and 2 of the drawings show a wooden piece made according to the invention in which the numeral 10 represents the body of the wooden piece completely covered or encased in a non-toxic, resilient, thin, dry and preferably non-tacky and non-glossy coating, skin or casing 12, which is preferably of such thickness as to be substantially invisible to the naked eye. As heretofore stated, an example of such coating or casing material comprises a natural unvulcanized rubber and methyl cellulose. Fig. 3 shows two such encased or coated wooden pieces being separated at 14 by the hands 15. The adhesive strength of coating 12 to its wooden body 10 is at least equal to, but preferably greater than the strength created by the pull, which is necessary to separate the two coated wooden pieces which were previously adhered to each other by pressure, and because of the non-coalescence of the coatings, when the pieces are separated, only the contacting faces of the coatings or casings will separate while no separation occurs between bodies 12 and the casings 10.

From the foregoing, it is evident that there has herein been provided as an article of manufacture a wooden piece completely covered with a coating or casing comprising natural unvulcanized rubber interspersed with a water soluble ether, the said unvulcanized rubber and water soluble ether being in such ratio whereby when two such wooden coated pieces are pressed together slightly they will adhere to each other without coalescence of the coating material of the two pieces, the coating adhering to the wooden piece with an adhesive strength at least equal to the pull necessary to separate the two pieces whereby the said pieces may be re-united and re-separated a great many times without impairing the coatings.

While the invention has been described with respect to particular embodiments or examples which give satisfactory results, it will be understood by those skilled in the art after understanding the invention, that various changes and modifications may be made without departing from the spirit and scope of the invention and it is intended, therefore, in the appended claims to cover all such changes and modifications.

Having thus described the invention, what is claimed as new and desired to secure by Letters Patent is:

1. As an article of manufacture, a wooden piece completely covered with a coating consisting essentially of natural unvulcanized rubber interspersed with a water soluble cellulose ether, the said natural unvulcanized rubber and the said water soluble cellulose ether being in such ratio whereby when two such wooden coated pieces are pressed together slightly they will adhere to each other without coalescence of the coating material of the two pieces, the coating adhering to the wooden piece with an adhesive strength at least equal to the pull necessary to separate the two pieces whereby the said pieces may be re-united and re-separated a great many times without impairing the said coatings.
2. As an article of manufacture, a wooden piece according to claim 1, and wherein said coating consists essentially of natural unvulcanized rubber and methyl cellulose.
3. As an article of manufacture, a wooden piece ac-

cording to claim 1, and wherein said coating is transparent, non-tacky, non-glossy and of such thickness as to be substantially invisible to the naked eye.

**References Cited in the file of this patent.**

**UNITED STATES PATENTS**

|           |               |               |
|-----------|---------------|---------------|
| 1,560,172 | Chamberlain   | Nov. 3, 1925  |
| 2,063,439 | Fischer       | Dec. 22, 1936 |
| 2,199,700 | Gramelspacher | May 7, 1940   |

|   |           |
|---|-----------|
| 5 | 2,279,256 |
|   | 2,498,403 |
|   | 2,586,009 |
|   | 2,586,039 |
|   | 2,644,280 |
|   | 2,699,999 |
|   | 376,531   |

|          |               |
|----------|---------------|
| Mark     | Apr. 7, 1942  |
| Elemdorf | Feb. 21, 1950 |
| Dickey   | Feb. 19, 1952 |
| Heggedal | Feb. 19, 1952 |
| O'Neill  | July 7, 1953  |
| Mahler   | Jan. 18, 1955 |

**FOREIGN PATENTS**

|       |         |
|-------|---------|
| Italy | of 1939 |
|-------|---------|